

March 26, 1935.

**A. H. HARRISON**

**1,995,540**

## METHOD OF AERATING SLURRIES.

Filed July 5, 1932



*Inventor.*  
ARTHUR HUGO HARRISON

ARTHUR HUGO HARRISON

BY  ATTORNEY.

Patented Mar. 26, 1935

1,995,540

XR

## UNITED STATES PATENT OFFICE

1,995,540

## METHOD OF AERATING SLURRIES

Arthur Hugo Harrison, Gold Pines, Ontario, Canada, assignor to Carbonated Lime Processes Limited

Application July 5, 1932, Serial No. 620,845

1 Claim. (Cl. 83—73) 259-147

This invention relates to the aeration of slurries in the production of porous building materials. It is applicable to cementitious materials, which have the inherent capacity to set and harden upon hydration, and equally well to materials, which have not in themselves this setting capacity but which require some further processing step to bind the aerated mass into permanent form, such, for example, as lime and clay, which may be hardened by carbonation and burning respectively.

Various methods of aerating cementitious materials have been proposed, among which may be mentioned the chemical release of a gas in the slurry, whipping air into the slurry, and mixing the premade foam therein. Some of these methods have been widely used in the production of porous building materials from plaster of Paris, cement and the like. In view of the greater insulation capacity of cellular materials these methods have made it possible to produce greatly improved building materials.

The object of the present invention is to provide an improved and simple method of aeration in making such cellular materials.

The invention will now be described with reference to the accompanying drawing which illustrates diagrammatically the operation of the method and in which,

Figure 1 is a longitudinal sectional view of the apparatus and

Figure 2 a cross sectional view on line 2—2 of Figure 1.

It has been found that air can be most successfully incorporated in a slurry by suitable agitation, beating or mixing in a closed space and that the density of the aerated product can be determined by the pressure maintained in the closed space during the agitation or mixing. As the air is whipped into the slurry the latter expands to occupy space originally filled with the air and when released from the chamber the aerated slurry expands as determined by the pressure maintained in the chamber. When the pressure in the closed space is varied the density of the aerated slurry and of the hardened or finished product made therefrom varies and adjustment of this pressure provides a ready means of regulating the density of the finished product.

In the drawing, 1 represents a chamber providing the closed space within which the aeration of the slurry is effected. 2 is a rotatable shaft carrying radial arms 3 on which are mounted a plurality of bars or paddles 4, the whole constituting the means for uniformly incorporating the air into the slurry. The shaft 2 is mounted in any suitable bearings and is caused to rotate at the desired rate by a motor or any suitable means, not shown. Helically set

vanes or other means 5 of any desired type are provided for causing the slurry to travel through the agitating zone at a rate such that the required amount of air will be incorporated in the slurry during the passage of the slurry through the agitating zone. The agitating arms 4 are preferably shorter than the chamber 1 so as to provide a feeding zone 6 and a discharge zone 7. Slurry is fed into the zone 6 by means of a pipe or the like 8 discharging near the bottom of the chamber. Air under a predetermined constant pressure is admitted at 9. The aerated slurry under the influence of the pressure in the chamber is discharged at 10. A pressure relief valve 11 may be provided.

In operation a slurry, comprising a mixture of water and cement, plaster of Paris, lime, clay or the like, and containing any suitable bubble-forming agent, is fed into the chamber and air at a desired pressure, which may vary from atmospheric up, is admitted. The relative volumes of air (calculated at atmospheric pressure) and unaerated slurry maintained in the chamber are preferably substantially as 2 to 1. There is always present an excess of air over that incorporated in the slurry and the pressure is kept constant throughout the operation while producing a cellular product of a given weight. Under the influence of the travelling paddle arms 4 air is drawn or whipped into the slurry, where it is retained in the form of bubbles by the bubble-forming agent. The period of agitation and the rate at which the shaft 2 travels will influence the amount of air incorporated in the slurry, but in practice these factors are preferably fixed at the most convenient point and the extent of aeration governed by the pressure maintained in the chamber. Increase in pressure increases the amount of air occluded in the slurry and, of course, when the aerated slurry is discharged from the chamber the mass expands with the freedom from super-atmospheric pressure.

The following specific examples are given to illustrate the effect of variation in the pressure within the chamber. In these cases the shaft of the agitating device was rotated at 270 R. P. M. and the period of agitation was two minutes.

1. A slurry of Portland cement was aerated as above described under the following conditions of pressure and the product weighed after being allowed to set for 10 days.

| Weight—lbs.                       |    |
|-----------------------------------|----|
| per cu. ft.                       | 55 |
| Agitation at atmospheric pressure | 65 |
| Agitation at 30 lbs. pressure     | 37 |
| Agitation at 50 lbs. pressure     | 25 |

2. A slurry of plaster of Paris aerated under 60

different pressures and weighed after setting for 2 days gave the following results.

|                                     | Weight—lbs.<br>per cu. ft. |
|-------------------------------------|----------------------------|
| 5 Agitation at atmospheric pressure | 68                         |
| Agitation at 12 lbs. pressure       | 62                         |
| Agitation at 24 lbs. pressure       | 51                         |
| Agitation at 60 lbs. pressure       | 23                         |

3. A lime slurry aerated as described gave the 10 following results.

|                                            | Weight—lbs.<br>per cu. ft. |
|--------------------------------------------|----------------------------|
| Slurry before agitation                    | 77.8                       |
| Slurry agitated under atmospheric pressure | 47.5                       |
| Agitation at 20 lbs. pressure              | 35.3                       |
| Agitation at 30 lbs. pressure              | 29.3                       |
| Agitation at 40 lbs. pressure              | 25.8                       |

4. A slurry of clay aerated under varying pressures gave the following results.

|                               | Weight—lbs.<br>per cu. ft. |
|-------------------------------|----------------------------|
| Slurry before agitation       | 81.5                       |
| Agitation at 30 lbs. pressure | 57.1                       |
| Agitation at 50 lbs. pressure | 33.4                       |
| Agitation at 83 lbs. pressure | 17.5                       |

These examples illustrate the fact that the 30 density of the product may be maintained at

the desired point by control of the air pressure employed during aeration. The rate at which the agitator revolves and the time of agitation are mentioned merely as illustrative of what has been done in this respect in practice and are subject to wide variation.

Bubble-forming agents of the character herein used are well known and there are many available. Rosin soap, glue and saponin may be mentioned as examples of some that may be used alone or in combination.

It will be apparent that aerated slurries of non-cementitious material, such as lime, clay and the like, require further processing to put them in the form in which they will be used in practice and such processes are now available in the art. The aerated lime slurry may be hardened by carbonation and the clay by burning.

I claim:

In the production of cellular building materials the method of aerating a slurry which comprises admitting slurry containing a bubble-forming agent to a closed space to but partially fill said space, admitting air to fill said space and to provide therein a predetermined pressure greater than atmospheric, maintaining said predetermined pressure constant and agitating the slurry to cause at least a portion of said air to be incorporated therein.

ARTHUR HUGO HARRISON.